

# UNITED STATES PATENT OFFICE.

CLIFFORD A. WOODBURY, OF CHESTER, PENNSYLVANIA.

## EXPLOSIVE.

1,149,487..

Specification of Letters Patent. Patented Aug. 10, 1915.

No Drawing.

Application filed January 14, 1914. Serial No. 811,938.

To all whom it may concern:

Be it known that I, CLIFFORD A. WOODBURY, of Chester, in the county of Delaware, and in the State of Pennsylvania, have invented a certain new and useful Improvement in Explosives, and do hereby declare that the following is a full, clear, and exact description thereof.

My invention relates particularly to the production of explosives and especially nitroglycerin explosives, which solidify only with difficulty and at very low temperatures and which have a low freezing point.

Nitroglycerin explosives as previously made freeze at a comparatively high temperature. They even freeze at a temperature above the freezing point of water. It therefore becomes necessary in using such explosives during a large part of the year to store the same in heated buildings and to use great care to keep them warm until they are loaded into the bore holes. Even then, it often happens that these explosives become frozen by contact with the cold walls of the bore holes. If the explosive should become frozen, many disadvantages result. There is always a loss of efficiency by the use of such explosives when frozen, inasmuch as they only detonate partially and frequently leave unexploded sticks of the explosive scattered through the rocks after the explosion. Attempts have been made in the past to produce low freezing explosives, but these have been only partially successful, either owing to the fact that the powder would still freeze too easily to offer any advantage over the grades of dynamite previously used or owing to the fact that the change in the constitution of the composition of the explosive rendered the explosive so insensitive as to be impracticable. Most of the low freezing explosives made up to the present time have depended for their alleged low freezing quality upon the presence of one or more organic nitro compounds such, for example, as nitrobenzene, nitrotoluene, etc. Some of these explosives had freezing points as low as 30° to 35° F., but these would readily freeze at lower temperatures such as, for example, between 15° to 20° F. In order for a low freezing explosive to be practicable, it is necessary for it to remain unfrozen for long periods of time at temperatures as low as 0° to 10° F.

I have discovered that a low freezing explosive can be produced that is far superior to any previously known by using as the base of the explosive a solution of a nitrated sugar in nitroglycerin to which has been added an organic nitro compound. I have discovered that the explosives made in this manner resist freezing to a remarkable extent, due to the fact that the mixture has a very low freezing point and due to the fact that the mixture because of certain physical properties remains liquid even when kept for long periods of time at temperatures far below its actual melting point. For example, a mixture of this kind which has an actual melting point of 30° F. will remain unfrozen for days or even weeks at temperatures as low as 0° to 10° F. These mixtures may be produced in many different ways but for the purpose of illustration I will describe certain ways in which they may be obtained. The mixing of these explosives may be accomplished in the same manner as the mixing of ordinary dynamite. The nitrated sugar and the organic nitro compounds may either be dissolved in the nitroglycerin before the latter is added to the remaining ingredients of the explosive, or they may be added to the other ingredients at the same time that the nitroglycerin is added. The remaining ingredients are such as are ordinarily used in the production of nitroglycerin dynamite, such for example as sodium or potassium nitrate, wood meal, etc. As one illustrative formula of such a composition I give the following:

|                     |      |
|---------------------|------|
| Nitroglycerin       | 30%  |
| Nitrated cane sugar | 4%   |
| Trinitrotoluene     | 10%  |
| Sodium nitrate      | 42%  |
| Wood meal           | 13%  |
| Chalk               | 1%   |
| Total               | 100% |

It is to be understood that this represents only one grade of the new type of explosive, and that the same may be made in all grades ordinarily obtainable of ordinary dynamite. It is understood, moreover, that if desired other ingredients may be added or example, by adding nitrocotton it is possible to make low-freezing gelatin powders of excellent quality. As an example of one of

these low-freezing gelatin powders I cite the following formula:

|    |                     |      |
|----|---------------------|------|
| 5  | Nitroglycerin       | 30%  |
|    | Nitrated cane sugar | 4%   |
|    | Trinitrotoluene     | 10%  |
|    | Nitrocotton         | 1%   |
|    | Sodium nitrate      | 41%  |
| 10 | Wood meal           | 13%  |
|    | Chalk               | 1%   |
|    | Total               | 100% |

Low-freezing gelatin powders of excellent quality may be made by adding to a mixture 15 of nitroglycerin, nitrated sugar and a nitro compound, a proper quantity of nitrocotton.

While I have described my invention above in detail, I wish it to be understood that many changes may be made therein 20 without departing from the spirit of my invention.

I claim:

1. An explosive containing nitroglycerin, a nitrated sugar and a nitro derivative of a hydrocarbon.
  2. An explosive containing nitroglycerin, a nitrated sugar and a nitro derivative of an aromatic hydrocarbon.
  3. An explosive containing nitroglycerin, a nitrated sugar, a nitro derivative of a hydrocarbon, and another nitrated carbohydrate.
  4. An explosive containing nitroglycerin, a nitrated sugar and a nitrotoluene.
  5. An explosive containing nitroglycerin, a nitrated sugar and trinitrotoluene.
  6. An explosive containing nitroglycerin, nitro-cotton, a nitrated sugar and a nitro derivative of a hydrocarbon.
  7. An explosive containing nitroglycerin, nitro-cotton, a nitrated sugar and a nitro derivative of an aromatic hydrocarbon.
  8. An explosive containing nitroglycerin, nitro-cotton, a nitrated sugar and a nitro toluene.
  9. An explosive containing nitroglycerin, nitro-cotton, a nitrated sugar and trinitrotoluene.
  - 45 10. An explosive containing nitroglycerin, nitrated cane sugar and a nitro derivative of a hydrocarbon.
- nitrated cane sugar and a nitro derivative of a hydrocarbon. 50
11. An explosive containing nitroglycerin, nitrated cane sugar and a nitro derivative of an aromatic hydrocarbon. 55
12. An explosive containing nitroglycerin, nitrated cane sugar, a nitro derivative of a hydrocarbon and another nitrated carbohydrate.
13. An explosive containing nitroglycerin, nitrated cane sugar and a nitrotoluene. 60
14. An explosive containing nitroglycerin, nitrated cane sugar and trinitrotoluene.
15. An explosive containing nitroglycerin, nitro-cotton, nitrated cane sugar and a nitro derivative of a hydrocarbon. 65
16. An explosive containing nitroglycerin, nitro-cotton, nitrated cane sugar and a nitro derivative of an aromatic hydrocarbon.
17. An explosive containing nitroglycerin, a nitrated sugar, a nitro derivative of an aromatic hydrocarbon, an oxygen-bearing salt and wood meal. 70
18. An explosive containing nitroglycerin, a nitrated sugar, trinitrotoluene, sodium nitrate and wood meal. 75
19. An explosive containing nitroglycerin, a nitrated sugar, a nitro derivative of an aromatic hydrocarbon, an oxygen-bearing salt and a combustible absorbent.
20. An explosive containing nitroglycerin, a nitrated sugar, trinitrotoluene, sodium nitrate and a combustible absorbent. 80
21. An explosive containing nitroglycerin, nitro-cotton, a nitrated sugar, a nitro derivative of an aromatic hydrocarbon, an oxygen-bearing salt and a combustible absorbent. 85
22. An explosive containing nitroglycerin, nitro-cotton, a nitrated sugar, trinitrotoluene, sodium nitrate and a combustible absorbent. 90

In testimony that I claim the foregoing I have hereunto set my hand.

CLIFFORD A. WOODBURY.

Witnesses:

ANNE GRAY TAYLOR,  
INEZ EARLE WOODBURY.

Copies of this patent may be obtained for five cents each, by addressing the "Commissioner of Patents, Washington, D. C."